

Aug. 16, 1932.

C. W. SWOPE

1,872,524

PROCESS FOR PRODUCING SHEET GLASS

Filed June 7, 1930

2 Sheets-Sheet 1



Inventor

Charles W. Swope.

By

Frank Fraser

Attorney

Aug. 16, 1932.

C. W. SWOPE

1,872,524

PROCESS FOR PRODUCING SHEET GLASS

Filed June 7, 1930

2 Sheets-Sheet 2



Inventor

Charles W. Swope.

By *Frank F. Swope*  
Attorney

## UNITED STATES PATENT OFFICE

CHARLES W. SWOPE, OF TOLEDO, OHIO, ASSIGNOR TO LIBBEY-OWENS-FORD GLASS COMPANY, OF TOLEDO, OHIO, A CORPORATION OF OHIO

## PROCESS FOR PRODUCING SHEET GLASS

Application filed June 7, 1930. Serial No. 459,645.

The present invention relates to a process for forming and annealing sheet or plate glass.

According to one process of manufacturing sheet glass, a plurality of successive sheets or plates of glass are intermittently rolled at predetermined intervals from a series of charges or masses of molten glass, the molten glass being preferably melted and refined within suitable receptacles or pots and poured therefrom onto a receiver from where it is moved to and passed between a pair of forming rolls which function to reduce the glass to a sheet of substantially predetermined and uniform thickness. In such process, it is desirable from both the standpoint of quality and production, that the glass sheets be formed at a relatively high rate of speed, after which the speed of travel thereof be materially reduced so that the sheets will be permitted to move at a relatively slower speed during annealing in order that the annealing apparatus need not be of an undesirable length. Also, in such process, it is desirable that the glass sheet be carried forwardly as it is formed at a relatively high rate of speed until it has become sufficiently set to support its own weight in order to prevent sagging of said sheet between the spaced rolls commonly employed for supporting the same. The carrying of the sheet forwardly at a high rate of speed until it becomes set requires the use of a conveying and/or annealing apparatus of considerable length, even though the time required in cooling be only a matter of a few minutes.

One of the objects, therefore, of this invention is the provision of a process whereby a mass of molten glass may be rapidly reduced to sheet form and the said sheet subsequently annealed while traveling at a relatively slower rate of speed.

Another object of the invention is the provision of a process wherein the speed of forward travel of the sheet may be reduced from

its relatively high forming speed to a relatively slower annealing speed easily and conveniently, while giving maximum support to the sheet to prevent sagging thereof.

A further object of the invention is the provision of a process wherein the sheet can be carried forwardly over a series of transverse supports at a relatively high rate of speed to prevent sagging thereof with a relatively slow forward movement in order that a relatively short conveying means may be used.

A further object of the invention is the provision of a process wherein the sheet is carried forwardly upon a series of supporting rolls movable bodily beneath the sheet preferably in a direction opposite to that of the travel thereof so as to more rapidly shift the lines of support from one position to another beneath the sheet, thereby leaving no portion of the sheet unsupported for any material interval of time and giving it substantially no opportunity to sag, each of the sheet supporting rolls being simultaneously rotated about its own axis in the same direction as the movement of the sheet.

Other objects and advantages of the invention will become more apparent during the course of the following description when taken in connection with the accompanying drawings.

In the drawings forming a part of this application and wherein like numerals are employed to designate like parts throughout the same,

Fig. 1 is a vertical longitudinal section through apparatus constructed in accordance with the present invention,

Fig. 2 is a plan view thereof,

Fig. 3 is a side elevation of the forward portion of the annealing leer, showing the means for mounting and driving a part of the sheet conveying mechanism, and

Fig. 4 is a section taken substantially on line 4—4 of Fig. 3.

Referring to the drawings, 5 designates a receiver or support adapted to receive thereupon a mass or charge of molten glass 6 which is to be reduced to sheet form, said glass being supplied to the receiver from a pot or receptacle 7. Associated with one end of the receiver are the sheet forming rolls 8 and 9 arranged relative to one another to create a sheet forming pass therebetween through which the molten glass is moved and reduced to a sheet 10 of substantially predetermined and uniform thickness. As pointed out above, it is desirable that the glass sheet be formed at a relatively high rate of speed and the rolls 8 and 9 are consequently rotated in a manner to rapidly reduce the mass of molten glass 6 to sheet form.

As the glass sheet 10 leaves the forming rolls, it passes downwardly over an inclined 20 apron or slab 11 and is subsequently deflected into the horizontal plane and carried forwardly into and through an annealing leer designated in its entirety by the numeral 12. Arranged within the leer are a series of horizontally aligned rolls 13 adapted to support and convey the glass sheet therethrough at a constant relatively slow speed, said rolls being driven from a motor 14 through suitable reduction gearing 15 and a sprocket chain 16 30 trained about sprockets (not shown) carried at the ends of said rolls. Of course, any other suitable type of driving means may be employed without departing from the spirit of the invention.

The leer rolls 13 are adapted to be driven at a constant relatively slow annealing speed which is materially less than the peripheral speed of the forming rolls 8 and 9 during the formation of the sheet. For example, the 40 leer rolls may be driven at from two to fifteen feet per minute while the sheet is formed at the rate of from forty to sixty feet per minute. Consequently, some means must necessarily be provided for effecting a reduction 45 in the forward speed of travel of the sheet after it has been formed and prior to its being delivered or passed onto the leer rolls 13. In order to accomplish this and the other 50 objects of the present invention, there is positioned within the forward end of the leer 12 between the forming mechanism and leer rolls 13 a pair of endless conveyors designated in their entirety by the numerals 17 and 18. Although two conveyors have been 55 here shown, it is to be understood that one or any number may be used as preferred. Also since each conveyor is of the same construction, a description of only one will be given.

60 Each conveying mechanism 17 and 18 comprises a series of spaced parallel rolls 19 which are arranged as closely adjacent one another as is practicable and which are mounted in the form of an endless belt, said belt being trained about the horizontally

spaced drums 20 and 21 mounted upon shafts 22 and 23 respectively at each end of which is carried a sprocket 24. Each roll 19 is carried upon a shaft 25 which projects at opposite ends through slots 26 formed in the side walls of the leer. The shaft 25 of each roll is journaled at each end within a roller bearing 27 adapted to run when the roll is in the upper horizontal run of the belt upon a fixed rail 28 extending longitudinally within the leer.

Arranged at opposite sides of the leer outwardly thereof are the endless chains 29 and 30, each consisting of a plurality of pivotally associated intermeshing and overlapping links, said chains being trained about the sprockets 24. To rotate the chains in unison, either shaft 22 or 23 may be positively driven from a motor 31 through suitable reduction gearing located in casing 32. The adjacent overlapping ends of the links forming the chains 29 and 30 are provided with aligned openings through which the projecting end portions of roll shafts 25 extend, as shown in Fig. 4, the links being held upon the shafts by nuts 33. In other words, the rolls 19 are connected in endless belt formation by the links which connect the adjacent roll shafts 25. Upon rotation of sprockets 24 to drive chains 29 and 30, the rolls 19 will be carried bodily along rails 28 with respect to the sheet 10 resting thereupon. During such travel, the roll shafts 25 are free to rotate within bearings 27 and, in order to also permit free rotation thereof, the said shafts are loosely mounted within bushings 34 arranged within the aligned openings through the chain links.

For the purpose of rotating each of the rolls 19 about its own individual axis in the direction of movement of the sheet while said rolls are being bodily moved in the opposite direction, there is mounted upon one end of each roll shaft 25 outwardly of the leer 12 a sprocket 35. Arranged above the sprockets 35 is an endless sprocket chain 36 trained at each end of its loop about a sprocket 37 carried by shaft 38 and driven from motor 39 through suitable reduction gearing located in casing 40. Upon rotation of sprockets 37, the endless chain 36 will engage sprockets 35 and rotate the rolls about their individual axes in a direction opposite to the direction in which they are being carried bodily. For the purpose of maintaining the chain 36 in engagement with sprockets 35, there may be provided a longitudinally extending plate or the like 41 carried by brackets 42, said plate holding the lower horizontal run of the chain 110 downwardly in engagement with said sprockets.

In carrying the invention into practice, and by way of illustration only, let us assume that a glass sheet 10, sixty feet in length, is adapted to be formed at approxi- 115 120 125

mately sixty feet per minute and annealed while traveling at the rate of ten feet per minute. In such case, the forming rolls 8 and 9 will be driven in such a manner that they will have a peripheral speed of sixty feet per minute, and the leer rolls 13 driven so that they will have a peripheral speed of ten feet per minute. During the formation of the sheet, it is preferred that the chains 29 and 30 be driven so as to move the rolls 19 bodily at fifty feet per minute in a direction opposite to the direction of movement of the sheet and that the sprocket chain 36 be simultaneously driven in the opposite direction at sixty feet per minute. Thus, since the rolls 19 are being carried bodily in one direction at fifty feet per minute and the chain 36 simultaneously moving in the opposite direction at sixty feet per minute, the said rolls will be driven about their individual axes at the rate of 110 feet per minute while the forward travel of the sheet over the rolls will be but sixty feet per minute or, in other words, equal to the speed of formation of the sheet. After the sheet has been formed and is completely received upon the conveyor 17, the speed of travel of the sprocket chain 36 is reduced to ten feet per minute which will effect a reduction in the forward speed of travel of the sheet to ten feet per minute so that the sheet will be discharged from the conveyor onto the leer rolls 13 at annealing speed. Of course, the speeds above mentioned are merely given by way of example only since any relative speeds may be used. In addition, the reduction in the speed of travel of the sheet can be effected in different ways such as by varying the speed of the chain 36 as above described, or in maintaining this speed constant and varying the speed of the chains 29 and 30, or by varying both. However, the above method of operation is desirable for the reason that at no time will it be necessary to completely stop either the bodily movement of the conveyor rolls 19 or the rotation thereof.

From the above, it will be apparent that there has not only been provided a process and apparatus whereby successive sheets of glass may be formed at a relatively high rate of speed and subsequently annealed while traveling at a relatively slower speed, but wherein this can be accomplished in an easy and convenient manner while, at the same time, giving maximum support to the sheet to prevent sagging thereof. Thus, the rolls 19 can be moved bodily so that no portion of the glass sheet will remain unsupported long enough to give it time to sag between the rolls. In other words, the lines of support formed by the upper surfaces of the series of rolls are being shifted from place to place so rapidly that practically a continuous support is provided for the lower

surfaces of the sheet. In addition, due to the simultaneous rotation of the rolls about their individual axes, the said rolls will have rolling contact with the sheet, thereby preventing sliding and slippage between said rolls and sheet.

It is to be understood that the form of the invention herewith shown and described is to be taken as the preferred embodiment of the same, and that various changes in the shape, size and arrangement of parts may be resorted to without departing from the spirit of the invention or the scope of the subjoined claims.

I claim:

1. The process of producing sheet or plate glass, which consists in intermittently forming successive sheets of glass by a rolling operation and at a relatively high rate of speed, receiving and carrying each sheet forwardly as it is formed upon a series of surfaces bodily movable with respect to the sheet and in a direction opposite to the forward movement thereof, in reducing the speed of forward travel of the sheet while upon said surfaces and while maintaining the said bodily movement of the surfaces relative to the sheet, and in then passing the sheet at such reduced speed into and through an annealing zone.

2. The process of producing sheet or plate glass, which consists in intermittently forming successive sheets of glass by a rolling operation and at a relatively high rate of speed, receiving and carrying each sheet forwardly as it is formed upon a series of continuously revolving surfaces having rolling contact with the sheet and being bodily movable relative thereto in a direction opposite to the forward movement thereof, in reducing the forward speed of travel of the sheet while upon said surfaces and while maintaining the said bodily movement of the surfaces relative to the sheet, and in then passing the sheet at such reduced speed into and through an annealing zone.

3. The process of producing sheet or plate glass, which consists in intermittently forming successive sheets of glass by a rolling operation and at a relatively high rate of speed, receiving and carrying each sheet forwardly as it is formed and at a speed substantially equal to its speed of formation upon a series of surfaces bodily movable with respect to the sheet so that the said sheet travels over said surfaces at a speed relatively greater than its speed of formation, in reducing the forward speed of travel of the sheet while upon said surfaces and maintaining a relatively greater speed of movement of the sheet over said surfaces, and in then passing the sheet at such reduced speed into and through an annealing zone.

4. The process of producing sheet or plate glass, which consists in intermittently forming successive sheets of glass by a rolling op-

eration and at a relatively high rate of speed, receiving and carrying each sheet forwardly as it is formed and at a speed substantially equal to its speed of formation upon a series 5 of continuously revolving surfaces having rolling contact with the sheet and being bodily movable relative thereto so that the said sheet travels over said surfaces at a speed relatively greater than its speed of formation, in 10 reducing the forward speed of travel of the sheet while upon said surfaces and maintaining a relatively greater speed of movement of the sheet over said surfaces, and in then passing the sheet at such reduced speed into 15 and through an annealing zone.

5. The process of producing sheet or plate glass, which consists in intermittently forming successive sheets of glass by a rolling operation and at a relatively high rate of speed, 20 receiving and carrying each sheet forwardly as it is formed and at a speed substantially equal to its speed of formation upon a series of spaced transverse supports bodily movable relative to the sheet and in a direction opposite to the forward movement thereof so that the said sheet travels over the supports at a speed relatively greater than its speed of formation, in reducing the forward speed of travel of the sheet while upon the supports 25 and maintaining a relatively greater speed of movement of the sheet over said supports, and in then passing the sheet at such reduced speed into and through an annealing zone.

6. The process of producing sheet or plate glass, which consists in intermittently forming successive sheets of glass by a rolling operation and at a relatively high rate of speed, receiving and carrying each sheet forwardly as it is formed and at a speed substantially 35 equal to its speed of formation upon a series of spaced transverse supports bodily movable relative to the sheet and in a direction opposite to the forward movement thereof so that the said sheet travels over the supports at a speed relatively greater than its speed of formation, in reducing the forward speed of travel of the sheet while upon the supports and maintaining a relatively greater speed of movement of the sheet over said supports, in 40 transferring the sheet at such reduced speed onto a second series of spaced transverse supports while maintaining the relatively high speed of travel of the sheet over said first mentioned transverse supports until the sheet 45 is entirely received upon said second series of supports, and in conveying the sheet upon the second series of supports through an annealing zone.

7. The process of producing sheet or plate glass, which consists in intermittently forming successive sheets of glass by a rolling operation and at a relatively high rate of speed, receiving each sheet as it is formed and carrying it forwardly at a speed substantially 50 equal to the speed of formation thereof

upon a series of continuously revolving surfaces bodily movable with respect to the sheet and in a direction opposite to the forward movement thereof so that the said sheet travels over said surfaces at a speed relative 70 to its speed of formation, then reducing the forward speed of travel of the sheet while upon said surfaces and while maintaining a substantially greater speed of movement of the sheet over said surfaces 75 until the sheet has become substantially set, and in then passing the sheet at such reduced speed from said surfaces into an annealing zone.

8. The process of producing sheet or plate glass, which consists in intermittently forming successive sheets of glass by a rolling operation and at a relatively high rate of speed, receiving and carrying each sheet forwardly as it is formed upon a series of continuously revolving supporting surfaces bodily movable with respect to the sheet and in a direction opposite to the forward movement thereof, reducing the forward speed of travel of the sheet while upon said surfaces and passing the sheet at such reduced speed from said surfaces into an annealing leir, and in maintaining at all times the speed of travel of the sheet over said supporting surfaces substantially greater than the speed of forward movement thereof.

9. The process of producing sheet or plate glass, wherein the sheet is formed at a relatively high rate of speed, carried forwardly 100 at its speed of formation for a predetermined distance, after which its speed of forward travel is reduced to a relatively slower speed, which consists in receiving and carrying each sheet forwardly as it is formed upon a series of surfaces revolving in the same direction as the forward movement of the sheet and being simultaneously bodily movable with respect to the sheet and in a direction opposite to the forward movement thereof so that the travel of the sheet over the surfaces is relatively greater than its forward movement, in reducing the speed of forward travel of the sheet while upon said surfaces, and concurrently maintaining the said bodily movement of the surfaces relative to the sheet, and in then passing the sheet at such reduced speed from said surfaces into an annealing zone.

10. The process of producing sheet or plate glass, wherein the sheet is formed at a relatively high rate of speed, carried forwardly 110 at its speed of formation for a predetermined distance, after which its speed of forward travel is reduced to a relatively slower speed, which consists in receiving and carrying each sheet forwardly as it is formed upon a series of surfaces revolving in the same direction as the forward movement of the sheet and being simultaneously bodily movable with respect to the sheet and in a direction opposite to the forward movement thereof so that the

travel of the sheet over the surfaces is relatively greater than its forward movement, in reducing the speed of forward travel of the sheet while upon said surfaces by varying the  
5 ratio of the speed between the revolving movement of the surfaces and the bodily movement thereof while maintaining the said bodily movement of the surfaces relative to the sheet, and in then passing the sheet at  
10 such reduced speed from said surfaces into an annealing zone.

Signed at Toledo, in the county of Lucas and State of Ohio, this 5th day of June, 1930.  
CHARLES W. SWOPE.

15

20

25

30

35

40

45

50

55

60